

# UNITED STATES PATENT OFFICE.

ANTONIO PIDELASERRA Y BRIAS AND MARIANO PIDELASERRA Y BRIAS, OF  
BARCELONA, SPAIN.

## MANUFACTURE OF COPYING-PAPER.

No. 901,824.

Specification of Letters Patent.

Patented Oct. 20, 1908.

Application filed March 13, 1908. Serial No. 420,840.

To all whom it may concern:

Be it known that we, ANTONIO PIDELASERRA Y BRIAS and MARIANO PIDELASERRA Y BRIAS, manufacturers, of Barcelona, Spain, residing at Barcelona, in the Province of Barcelona and Kingdom of Spain, have invented certain new and useful Improvements in the Manufacture of Copying-Paper; and we do hereby declare the following to be a full, clear, and exact description of the invention, such as will enable others skilled in the art to which it appertains to make and use the same.

There are well known in the art of paper manufacture some papers specially prepared so as to retain a certain moisture which permits of their taking copies by means of the ordinary presses and copying machines usually employed in the commercial offices, without previously moistening the paper. To this end, said papers are impregnated with a solution of an hygroscopic salt with or without glycerin, or they are impregnated with a mere solution of glycerin more or less diluted in water according to the effect to be produced. While these papers may take press-copies more or less neat and perfect according to the preparation they have undergone and also according to the means adopted for copying; yet it is well known that the dampness that they possess causes the ink to spread in the paper and there will come a time when it will not be possible to read these copies. On the other hand, the constant moisture of the paper makes it less durable and offers great objections to the handling of the sheets or leaves, either when turning them over to find a given copy, or when choosing the sheets to take them out and keep them in the files with other documents; because the paper so prepared does not prove resistant enough and becomes injured very easily.

It has been found in practice that the paper should have as little moisture as possible to take the ink well, and its touch should be the same as dry paper. These results may be obtained by adding the solution of glycerin or of hygroscopic salt in so small a quantity that the paper cannot take press-copies in the ordinary copying presses; but will require a very heavy pressure to take neat copies thereon. In order to fix the ink, the glycerin bath or the solution of an hygroscopic salt, is prepared with a solution of

gallic acid which renders the paper able to fix the ink when taking the copy and therefore the ink or color does not spread at all; but the copies will remain neat and inalterable whatever may be the time elapsed. The percentage of gallic acid added to the solution depends on the effect to be produced. A too heavy percentage of gallic acid would soak into the original writing and so fix the ink therein that no more copies could be taken thereof.

In order to give the paper a dry touch and the necessary strength to be easily manifolled and to prove as durable as the ordinary copying paper (which needs to be previously moistened for copying), to the bath above referred to is added a quantity of saponified wax and honey. We mean by "saponified wax" the product obtained by adding wax in the saponifying process, or the product obtained by mixing soap and wax in equal parts and heating them together in a suitable receptacle. The proportions of these ingredients are variable but experience has shown that with a 2 per cent. saponified wax and a 15 per cent. honey added to the bath, good results may be obtained. The class of paper which lends itself best to that use, is woodpulp paper. The time of passage of the paper through the bath should not exceed the time just necessary for the absorption of the liquid, when it is dried and then calendered or cylindered. The paper thus obtained is bright, strong and durable.

For the wax and honey may be substituted other materials which can impart to the paper similar properties. Instead of wax, we may employ for instance ceresin, stearin, tallow, or other like materials; and in lieu of honey we may employ sugar, molasses, glucose, or the like. Instead of gallic acid we may choose some other acid among those usually employed for fixing colors.

The moistening operation or passage of the paper in the bath is carried out with the paper in sheets or in endless bands, and also by the same or similar means or machines that are usually employed in paper manufacture or in similar industries.

It will thus be seen that the glycerin or hygroscopic salt serves to hold enough moisture in the paper to effect the copying process; that the saponified wax and honey

serve to give the paper a dry touch and to prevent its tearing when handled; and that the gallic acid readily combines with the ink of the paper to be copied, serving to soften 5 the same, to make it more acid, and to fix it and thereby prevent it from spreading.

What we claim is:—

1. The process of producing copies from impressions made in ink which consists in 10 impregnating a suitable sheet of paper with a compound capable of taking up moisture to which has been added an acid, and a saponified wax; in bringing said sheet in contact with the impressions to be copied; 15 and applying sufficient pressure to cause a copy to be taken, substantially as described.

2. The method of preparing sheets of paper for use in copying, which consists in saturating said sheets with a solution con- 20 taining a hygroscopic compound to which

has been added gallic acid and saponified wax, substantially as described.

3. The method of preparing sheets of paper for use in copying, which consists in impregnating said sheets with a solution con- 25 taining glycerin, gallic acid, saponified wax, and honey, substantially as described.

4. The method of preparing sheets of paper for use in copying, which consists in impregnating said sheets with a solution 30 containing glycerin, gallic acid, saponified wax, and honey, and then calendering said paper, substantially as described.

In testimony whereof, we affix our signatures, in presence of two witnesses.

ANTONIO PIDELASERRA Y BRIAS.  
MARIANO PIDELASERRA Y BRIAS.

Witnesses:

STANLEY C. HARRIS,  
CONSTANTINO LUPER CID.